

# United States Patent [19]

Willems et al.

[11] 3,808,005

[45] Apr. 30, 1974

[54] **SILVER HALIDE EMULSION STABILIZED WITH A BIDENTATE HETEROCYCLIC COMPOUND CONTAINING A SULPHO OR A CARBOXYL GROUP**

[75] Inventors: **Jozef Frans Willems, Wilrijk; Frans Clement Heugebaert, Kontich; Robert Joseph Pollet, Berchem, all of Belgium**

[73] Assignee: **AGFA-Gevaert N.V., Mortsel, Belgium**

[22] Filed: **May 10, 1971**

[21] Appl. No.: **141,995**

## Related U.S. Application Data

[63] Continuation-in-part of Ser. No. 795,077, Jan. 29, 1969, abandoned.

## Foreign Application Priority Data

Feb. 22, 1968 Great Britain ..... 8653/68

[52] U.S. Cl. ..... **96/76 R, 96/109**

[51] Int. Cl. ..... **G03c 1/34, G03c 1/48**

[58] **Field of Search** ..... 96/109, 76 R

## [56] References Cited

### UNITED STATES PATENTS

|           |        |                    |          |
|-----------|--------|--------------------|----------|
| 3,137,578 | 6/1964 | De Selms .....     | 96/109   |
| 3,305,362 | 2/1967 | Riester et al..... | 96/109 X |
| 3,042,521 | 7/1962 | Deysch et al. .... | 96/109 X |

*Primary Examiner*—J. Travis Brown

*Assistant Examiner*—Won H. Lovie, Jr.

*Attorney, Agent, or Firm*—A. W. Breiner

## [57] ABSTRACT

Photographic materials comprising a light-sensitive silver halide emulsion and containing a stabilizer against formation and growth of fog are described. The stabilizer is a bidentate heterocyclic compound having at least two nitrogen coordinating atoms for silver and a water-solubilizing carboxyl or sulphogroup. Fog growth is prevented without inhibiting emulsion sensitivity.

**6 Claims, No Drawings**

**SILVER HALIDE EMULSION STABILIZED WITH A BIDENTATE HETEROCYCLIC COMPOUND CONTAINING A SULPHO OR A CARBOXYL GROUP**

The present application is a continuation-in-part of Application Ser. No. 795,077 filed Jan. 29, 1969 now abandoned.

This invention relates to improved photographic materials comprising light-sensitive silver halide emulsions and more particularly to photographic materials having less tendency to fog formation while still possessing the same light-sensitivity.

It is well known that light-sensitive silver halide materials comprising gelatin silver halide emulsion layers are subject to fogging. Fogging in general and chemical fogging in particular may be defined as the formation of a uniform deposit of silver on development which is dependent on a whole series of circumstances and factors namely on the nature of the emulsions, on their age, on the conditions under which they have been stored, on the development conditions, etc. For particular development conditions the fog tends to be greater as the time of storage and the temperature and relative humidity of the atmosphere in which the emulsions are stored are increased. Consequently it is known to carry out accelerated tests called "incubation" tests on the stability of photographic emulsions by storing them at elevated temperature and humidity and then determining their sensitometric characteristics.

Addenda to the photographic material known as stabilizers or antifoggants protect the light-sensitive silver halide emulsions against formation and growth of fog particularly in highly sensitive emulsions and in emulsions which are to be stored under conditions of high temperature and humidity as is for instance the case in tropical countries.

It is well known to use compounds of the triazolopyrimidine type (azaindolizines) as stabilizers for light-sensitive photographic silver halide emulsions. Although these compounds are very effective stabilizers, emulsions containing them still show a tendency to fog formation in extreme storage circumstances i.e. at very high temperatures and humidities and in extreme development circumstances e.g. rapid processing at elevated temperatures.

It is also known from U.S. Patent specification No. 3,137,578 to protect light-sensitive silver halide emulsions against the growth of chemical fog during storage by addition of benzimidazoles substituted in the 2-position by a 2-pyrrolylgroup, a 2-furylgroup, a 2-thienylgroup, a 2-pyranyl group, a 2-thiopyranyl group, a 2-tetrahydropyranylgroup, a 2-tetrahydrofuryl group, a 2-tetrahydrothiopyranyl group and the like heterocyclic groups.

These compounds, however, have but a very low fog-inhibiting effect and reduce the emulsion sensitivity markedly.

It has now been found that heterocyclic bidentate reagents for silver comprising at least one water-solubilizing group and more particularly compounds corresponding to the following general formula:



wherein:

R stands for hydrogen or lower alkyl comprising at most four carbon atoms including substituted lower alkyl,

Z represents the atoms necessary to complete a heterocycle including a substituted heterocycle and a heterocycle with fused ring e.g. imidazole, benzimidazole, naphthimidazole, imidazopyridine, imidazoline, pyrazole, triazole, tetrazole, etc.

A stands for a chemical bond, alkylene such as methylene, ethylene, tetramethylene etc. including alkylene interrupted by oxygen or a  $-\text{N}(\text{R})-$  group wherein R has the same significance as above, arylene, alkenylene, such as vinylene and  $-\text{S-alkylene-S-}$  or  $-\text{S-alkylene-}$  the alkylene groups of which can be interrupted by oxygen or a  $-\text{N}(\text{R})-$  group wherein R has the same significance as above,

X stands for a heterocycle including a substituted heterocycle and a heterocycle with fused ring, said heterocycle comprising the moiety  $=\text{N}-$ , for example imidazole, benzimidazole, naphthimidazole, imidazopyridine, imidazoline, pyrazole, pyridine, quinoline, thiazole, tetrazole, triazole, etc., and

wherein a water-solubilizing group, more particularly a  $-\text{COOM}$  or  $-\text{SO}_3\text{M}$  group with M = hydrogen, ammonium, a metal atom, an organic amine, etc., is linked directly or indirectly to the grouping Z and/or X and/or A, are particularly good stabilizers and antifoggants for photographic light-sensitive silver halide emulsions without causing an objectionable desensitization of the light-sensitive material.

Moreover, it has been found that the compounds according to the invention are very suitable for use in combination with stabilizers of the triazolopyrimidine type, particularly in extreme storage and development circumstances in order to reduce the fogging tendency of the light-sensitive emulsion without giving rise to an appreciable desensitization thereof.

The compounds corresponding to the above general formula are referred to as being bidentate heterocyclic compounds which means that they are bidentate ligands for forming complexes with silver i.e. they should contain at least two coordinating atoms for silver, the nitrogen atom of the



group of the heterocycle being one of the coordinating atoms and the nitrogen atom of the  $=\text{N}-$  moiety in X being the other coordinating atom. Thus, the moiety  $=\text{N}-$  in X is an essential feature of the compounds of the invention.

The presence of (a) water-solubilizing group(s) is also an essential feature of the compounds of the invention since compounds corresponding to the above general formula but containing no water-solubilizing group generally have a markedly less stabilizing action more particularly a marked desensitizing effect.

The compounds having the structures listed below are representative of those falling within the scope of the above general formula.



3



4



28.



29.



30.



31.



The above specific compounds can be prepared as illustrated by the following preparations:

**Preparation 1 : Compound 1**

2-(2-imidazolyl)-5-sulphoimidazole was prepared by sulphonation of 2,2'-diimidazole according to J.prakt. Chem. 24, 164 (1964).

**Preparation 2 : Compound 2**

60 g (0.307 mole) of 2-(3-pyridyl)benzimidazole were added with stirring to 150 ccs (2.3 moles) of chlorosulphonic acid and the mixture was stirred for 8 hours. The reaction mixture was poured into 1 kg of ice-water. The 2-(3-pyridyl)-5(6)-chlorosulphonylbenzimidazole formed separated in the form of an oil. The sulphochloride was hydrolyzed by boiling and the crystalline product formed upon cooling in ice was recrystallized from water. Yield : 22 g of 2-(3-pyridyl)-5(6)-sulphobenzimidazole.  $\frac{1}{2}$  hydrate.

**Preparation 3 : Compound 3**

A mixture of 18 g (0.08 mole) of 2-carboxy-5-sulphopyridine and 8.64 g (0.08 mole) of o-phenylenediamine was heated for 6 hours at 160°C in 25 g of polyphosphoric acid. After having been cooled the mixture was poured into 200 ccs of ice-water and the precipitate formed was filtered by suction and redissolved in 100 ccs of 1N sodium hydroxide. The solution was acidified by means of hydrochloric acid whereby 13 g of 2-(5(6)-sulpho-2-pyridyl) benzimidazole precipitated.

**Preparation 4 : Compound 4**

12.3 g (0.1 mole) of picolinic acid and 18.8 g (0.1 mole) of 3,4-diaminobenzenesulphonic acid were heated for 6 hours at 200°C in 50 g of polyphosphoric acid. After having been cooled the mixture was poured into 300 ccs of water whereupon the precipitate formed was filtered by suction and recrystallized from water. Yield : 19 g of 2-(2-pyridyl)-5(6)-sulphobenzimidazole.  $\frac{1}{2}$  hydrate.

**Preparation 5 : Compound 5**

12.3 g (0.1 mole) of isonicotinic acid and 18.8 g (0.1 mole) of 3,4-diaminobenzenesulphonic acid were heated for 6 hours at 200°C in 50 g of polyphosphoric acid. After having been cooled the reaction mixture was poured into 300 ccs of water whereupon the precipitate formed was filtered by suction and recrystallized from water. Yield : 22 g of 2-(4-pyridyl)-5(6)-sulphobenzimidazole.  $\frac{1}{2}$  phosphoric acid.

**Preparation 6 : Compound 6**

227 g (1.16 mole) of 2-(4-pyridyl)benzimidazole were added with stirring to 567 ccs (8.7 mole) of chlorosulphonic acid whereupon the mixture was refluxed for 8 hours. The reaction mixture was poured into 4 kg of ice-water. The 2-(4-pyridyl)-5(6)-chlorosulphonylbenzimidazole separated in the form of a brown oil.

The sulphochloride was hydrolyzed by boiling and the pH of the solution obtained was adjusted to pH 2 by means of sodium carbonate. The reaction mixture was kept overnight at 0°C and the crystallized product was filtered by suction and then recrystallized from water. Yield : 207 g of 2-(4-pyridyl)-5(6)-sulphobenzimidazole monohydrate.

**Preparation 7 : Compound 7**

a. A solution of 18.8 g (0.1 mole) of 3,4-diaminobenzenesulphonic acid and 5.9 g (0.05 mole) of succinic acid in 150 ccs of 6N hydrochloric acid was refluxed for 12 hours. The mixture was concentrated by evaporation and the residue was washed with 250 ccs of water. Yield: 16 g of 1,2-bis(5(6)-sulpho-2-benzimidazolyl)-ethane.

b. This compound can also be prepared as described in Swiss Patent Specification 235,570 by sulphonation of 1,2-bis-2-(benzimidazolyl)-ethane with fuming sulphuric acid.

**Preparation 8 : Compound 8**

A solution of 18.8 g (0.1 mole) of 3,4-diaminobenzenesulphonic acid and 6.6 g (0.05 mole) of glutaric acid in 150 ccs of 6N hydrochloric acid was refluxed for 12 hours. The precipitate formed was filtered by suction and washed with 200 ccs of water. Yield : 14.5 g of 1,3-bis(5(6)-sulpho-2-benzimidazolyl)propane.

**Preparation 9 : Compound 9**

To a solution of 18 g (0.06 mole) of 1,4-bis(2-benzimidazolyl)-butane in 180 ccs of sulphuric acid were added dropwise 54 g of fuming sulphuric acid (24 percent of SO<sub>3</sub>). The reaction mixture was kept between 70° and 80°C until a sample taken dissolved completely in a solution of sodium carbonate. The reaction mixture was poured into ice-water and the precipitate formed was filtered by suction. The white powder formed was purified by dissolving it in sodium carbonate and then precipitating it by means of acetic acid. Yield : 19 g of 1,4-bis(5(6)-sulpho-2-benzimidazolyl)butane.

**Preparation 10 : Compound 10**

8.35 g (0.05 mole) of 2,6-pyridinedicarboxylic acid and 18.8 g (0.1 mole) of 3,4-diaminobenzenesulphonic acid were heated for 6 hours at 200°C in 50 g of polyphosphoric acid. After having been cooled the mixture was poured into 300 ccs of water, the precipitate formed was filtered by suction and washed with 200 ccs of water. Yield : 22 g of 2,6-bis(5(6)-sulpho-2-benzimidazolyl) pyridine monohydrate.

**Preparation 11 : Compound 11**

12.3 g of picolinic acid and 23.4 g of 3-amino-4-ethylaminobenzenesulphonic acid were heated for 6 hours at 200°C in 50 g of polyphosphoric acid. After having been cooled the reaction mixture was poured into 300 ccs of water, the precipitate formed was filtered by suction and recrystallized from water. Yield : 6 g of 1-ethyl-2-(2-pyridyl)-5(6)-sulphobenzimidazole.

## Preparation 12 : Compound 12

14.9 (0.1 mole) of 2-(2-pyridyl)acrylic acid and 18.8 g (0.1 mole) of 3,4-diaminobenzenesulphonic acid were heated for 6 hours at 200°C in 50 g of polyphosphoric acid. After having been cooled the reaction mixture was poured into 300 ccs of water and the precipitate formed was recrystallized from 300 ccs of 1N hydrochloric acid. Yield : 24.5 g of 2-[ $\beta$ -(2-pyridyl)-vinyl]-5(6)-sulphobenzimidazole hydrochloride monohydrate.

## Preparation 13 : Compound 13

10 g (0.036 mole) of 2-(5-sulpho-2-pyridyl)benzimidazole were added with stirring to 41.5 g (0.27 mole) of chlorosulphonic acid and the mixture was refluxed for 8 hours. The reaction mixture was poured into 150 g of ice-water and the solution was refluxed for 1 hour. By addition of a saturated solution of barium hydroxide, barium sulphate was precipitated. The barium sulphate was filtered by suction and washed with water. The filtrates were conducted over beads of insoluble-sulphonated polystyrene as cation exchanger. The eluate is evaporated till dry and the residue was recrystallized from ethanol. Yield : 2 g of 2-(5-sulpho-2-pyridyl)-5(6)-sulphobenzimidazole dihydrate.

## Preparation 14 : Compound 14

23.8 g of 3,4-diaminonaphthalenesulphonic acid and 12.3 g of 2-pyridinecarboxylic acid were dissolved in 100 g of polyphosphoric acid and heated for 6 hours at 200°C. After having been cooled the reaction mixture was poured into water and the precipitate formed was filtered by suction. The precipitate was redissolved in alkali and precipitated again by acidification whereupon it was recrystallized from water. Yield : 17 g of 2-(2-pyridyl)-7-sulpho-1H-naphtho[1,2-d]imidazole.

## Preparation 15 : Compound 15

17 g of N,N-bis[2-benzimidazolyl]-methylamine were dissolved in 109 g of chlorosulphonic acid. The mixture was refluxed for 15 hours and poured into ice-water. The precipitate formed was filtered by suction, redissolved in alkali, filtered over decolourizing carbon and acidified. Yield : 15 g of N,N-bis(5(6)-sulpho-2-benzimidazolylmethyl)-methylamine.

## Preparation 16 : Compound 16

18.8 g of 3,4-diaminobenzenesulphonic acid and 17.3 g of 2-quinolinecarboxylic acid were dissolved in 50 g of polyphosphoric acid and heated for 6 hours at 200°C. After having been cooled the reaction mixture was poured into water, the precipitate formed was filtered by suction and redissolved in alkali. The product was precipitated by acidification and the precipitate was recrystallized from water. Yield : 15 g of 2-(2-quinolyl)-5(6)-sulphobenzimidazole.

## Preparation 17 : Compound 17

A mixture of 2-(2-benzimidazolyl)-3H-imidazo[4,5-b] pyridine prepared as described in J.Chem.Soc. 33 (1967) and 25 ccs of chlorosulphonic acid was heated for 8 hours on a steam bath whereupon the reaction mixture was poured into ice-water. The sulphonyl chloride formed was refluxed for 8 hours in 100 ccs of concentrated hydrochloric acid. The precipitate formed upon cooling was filtered by suction. Yield : 5 g of 2-(5(6)-sulpho-2-benzimidazolyl)-3H-imidazo[4,5-b]pyridine.

## Preparation 18 : Compound 18

A mixture of 11 g of 2-(4-thiazolylmethyl)-benzimidazole prepared as described in Bull.Soc. Chim.France 1966, 1545 and 25 ccs of chlorosulphonic acid was heated for 8 hours on a steam bath whereupon it was poured into ice-water. The sulphonyl chloride formed was refluxed for 8 hours in 100 ccs of concentrated hydrochloric acid. The precipitate formed upon cooling was filtered by suction. Yield : 6 g of 2-(4-thiazolylmethyl)-5(6)-sulphobenzimidazole.

## Preparation 19 : Compound 19

3-sulpho-5-(4-pyridyl)-1H-1,2,4-triazole was prepared as described in J.Chem.Soc. (1967), 661.

## Preparation 20 : Compound 20

2-(2- $\Delta_2$ -imidazolyl)-5(6)-sulphobenzimidazole was prepared as described in J.Chem.Soc. (1967) 33.

## Preparation 21 : Compound 21

To a solution of 11.4 g of 1,2-bis-(5-mercaptop-1H-1,2,4-triazole-3-yl)ethane prepared as described in Bull. Soc.Chim.Belg. 75, 358 (1966) and 12 g of sodium methylate in 150 ccs of methanol 18 g of propanesultone were added. The mixture was refluxed for 3 hours and then filtered over decolourizing carbon. The filtrate was concentrated by evaporation and the residue was dissolved in ethanol. The product was precipitated by means of acetone. Yield : 22 g of 1,2-bis[5-(3-sulphopropylthio)-1H-1,2,4-triazol-3-yl]-ethane di-sodium salt.

## Preparation 22 : Compound 22

To a solution of 11.4 g of 1,2-bis(5-mercaptop-1H-1,2,4-triazol-3-yl)-ethane and 12 g of sodium methylate in 150 ccs of methanol, 20 g of 1,1,3-trimethylpropane-sultone were added. The mixture was refluxed for 3 hours and filtered over decolourizing carbon. The filtrate is concentrated by evaporation and the residue dissolved in ethanol. The product was precipitated by means of acetone. Yield : 30 g of 1,2-bis[5-(1,3-dimethyl-3-sulpho-butylthio)-1H-1,2,4-triazol-3-yl]-ethane disodium salt.

## Preparation 23 : Compound 23

44 g of 3-phenyl-5-(2-pyridyl)-pyrazole prepared as described in J.prakt.Chem., Vol. 34 (1966) 64, and 116 g of chlorosulphonic acid were refluxed for 8 hours. The reaction mixture was poured into water and the precipitate filtered by suction. It was redissolved in water and the solution formed was refluxed for 1 hour. The solution was concentrated by evaporation and the residue formed recrystallized from aqueous isopropanol. Yield : 9 g of 3-(m-sulphophenyl)-5-(2-pyridyl)-pyrazole.

## Preparation 24 : Compound 24

27.4 g of the disodium salt of 2-mercaptop-5(6)-sulphobenzimidazole and 17 g of 2-chloromethylbenzimidazole were suspended in 250 ccs of dimethyl formamide and heated with stirring for 6 hours at 70°C. The reaction mixture was evaporated till dry, and the residue was taken up in alkali. The solution was filtered over decolourizing carbon and acidified. The precipitate formed was recrystallized from water. Yield : 7 g of 2-(2-benzimidazolylthio)-5(6)-sulphobenzimidazole.

## Preparation 25 : Compound 25

To a solution of 7.5 g of 5-(4-pyridyl)-1H,1,2,4-triazole-3-thiol prepared as described in Rec.Trav.-Chim. Pays-Bas 73 (1954) 113, and 2.27 g of sodium methylate in 250 ccs of methanol, 5.12 g of propanesul-

tone were added. The mixture was refluxed for 4 hours and evaporated till dry. The residue was dissolved in water, filtered and acidified. The precipitate formed was recrystallized from water. Yield : 5.5 g of 3-(3-sulphopropylthio)-5-(4-pyridyl)-1H-1,2,4-triazole.

Preparation 26 : Compound 26

1,2-bis-(2-benzimidazolyl)-ethanesulphonic acid sodium salt was prepared as described in United States Patent specification No. 3,057,857.

Preparation 27 : Compound 27

To a suspension of 37.8 g of the sodium salt of 2-mercaptop-5-sulphobenzimidazole in 100 ml of water, a solution of 12 g of sodium hydroxide in 60 ml of water was added with stirring so that the benzimidazole compound dissolved completely.

At room temperature, a solution of 17.75 g of 5-chloromethyltetrazole in 100 ml of water was added dropwise in 15 minutes. The mixture was heated for 2 hours at 75°C and then cooled. The solution obtained was diluted with water to make 2 litres and then passed over an ion-exchanger. The solution was concentrated by evaporation, the residue recrystallized from 1 litre of dimethylformamide, filtered off, washed with ethanol and ether and dried at 100°C in vacuum. Yield : 35 g.

Preparation 28 : Compound 28

27.4 g of the disodium salt of 2-mercaptop-5(6)-sulphobenzimidazole and 12.8 g of 2-chloromethylpyridine were suspended in 200 ccs of dimethylformamide and heated for 6 hours with stirring at 80°C. The sodium chloride formed was filtered off by suction, whereupon the solution was evaporated till dryness. The residue was dissolved in water and acidified with acetic acid. Yield : 11 g of 2-(2-pyridylmethylthio)-5(6)-sulphobenzimidazole.

Preparation 29 : Compound 29

To a solution of 18 g of 1,3-bis-(5-mercaptop-1H-1,2,4-triazol-3-yl)-propane and 8 g of sodium methylate in 200 ccs of methanol, a solution of 18 g of propane-sultone in 300 ccs of methanol was added. The mixture was refluxed for 4 hours and evaporated till dryness. The residue was dissolved in water and conducted over an ion exchanger. The eluate is once again evaporated till dryness and the residue is recrystallized from water. Yield : 10 g.

Preparation 30 : Compound 30

To a solution of 18 g of 1,3-bis(5-mercaptop-1H-1,2,4-triazol-3-yl)-propane in 300 ccs of water an aqueous potassium permanganate solution was added dropwise until the colour did not disappear any more. The solution was filtered, conducted over an ion exchanger and evaporated. The residue was recrystallized from water. Yield : 9 g.

Preparation 31 : Compound 31

27.4 g of the disodium salt of 2-mercaptop-5(6)-sulpho-benzimidazole and 8.7 g of dibromomethane were suspended in 200 ccs of dimethylformamide and heated with stirring for 3 hours at 100°C. The solution was filtered and concentrated by evaporation. The residue was washed with methanol and recrystallized from a mixture of ethanol and water. Yield : 8 g.

The antifoggants according to the present invention are generally incorporated into the silver halide emulsion layer of the light-sensitive material. The way in which the compounds of use according to the invention

are added to emulsions is not critical and the addition can be made during any the emulsion preparation; they can be added before or after the emulsion has been optically sensitized, preferably just before coating of the emulsion on a suitable support such as for example paper, glass or film.

Instead of incorporating the compounds of the invention into the emulsion layer they can also be incorporated into another layer of the photographic material, e.g. a gelatin antistress layer or intermediate layer, which is in water-permeable relationship with the said emulsion layer or into one of the processing baths for said photographic material.

The antifoggants of use according to the present invention may be incorporated into any type of light-sensitive material comprising a silver halide emulsion layer e.g. a spectrally sensitized or non-sensitized silver halide emulsion layer, a silver halide emulsion layer of use in diffusion transfer processes for the production of silver images, an X-ray emulsion layer, and an emulsion layer sensitive to infra-red radiation. They may be incorporated into high speed negative materials as well as into rather low speed positive materials. Various silver salts may be used as the light-sensitive salt e.g. silver bromide, silver iodide, silver chloride, or mixed silver halides e.g. silver chlorobromide or silver bromoiodide.

The silver halides are dispersed in the common hydrophilic colloids such as gelatin, casein, zein, polyvinyl alcohol, carboxymethylcellulose, alginic acid, etc., gelatin being, however, favoured.

The amount of antifoggant employed in the light-sensitive silver halide material depends on the particular type of emulsion and the desired effect and can vary within very wide limits. The optimum amount of antifoggant to be added is best determined for each particular type of emulsion by trial. Generally, the most suitable concentration is between 0.2 millimole and 30 millimoles of antifoggant per mole of silver halide.

The light-sensitive emulsions may be chemically as well as optically sensitized. They may be chemically sensitized by effecting the ripening in the presence of small amounts of sulphur containing compounds such as allyl thiocyanate, allyl thiourea, sodium thiosulphate, etc. The emulsions may also be sensitized by means of reductors for instance tin compounds as described in our United Kingdom Patent specification No. 789,823 and small amounts of noble metal compounds such as gold, platinum, palladium, iridium, ruthenium and rhodium.

Other addenda such as hardening agents, wetting agents, plasticizers, colour couplers, developing agents and optical sensitizers can be incorporated into the emulsion in the usual way.

The antifoggants according to the present invention are particularly suitable for use in conjunction with compounds which sensitize the emulsion by development acceleration for example alkylene oxide polymers. These alkylene oxide polymers may be of various types. Various derivatives of alkylene oxides may be used to sensitize the silver halide emulsions e.g. alkylene oxide condensation products as described in United States Patent specification Nos. 2,531,832 and 2,533,990, in United Kingdom Patent specifications Nos. 920,637 — 940,051 — 945,340 and 991,608 and in Belgian Patent Specification 648,710. Other compounds that sensitize the emulsion by development acceleration and that are suitable for use in combination

with the antifoggants of use according to the invention are the onium derivatives of amino-N-oxides as described in Belgian Patent specification No. 686,520.

The stabilizers according to the invention can also be used in conjunction with other known stabilizers for instance with heterocyclic nitrogen containing thioxo compounds such as benzothiazoline-2-thione and 1-phenyl-Δ2-tetrazoline-5-thione, with mercury compounds such as those described in Belgian Patent Specifications 524,121, 677,337, 707,386 and 709,195 and as mentioned above, preferably with compounds of the hydroxytriazolopyrimidine type (hydroxyazaindolizines), particularly in extreme storage and development circumstances.

the table below in a concentration of 0.001 mole per kg of emulsion. Then the emulsions were coated on a conventional support and dried.

The values of speed, gradation and fog of the materials formed were determined shortly after preparation and after incubation for 5 days at 57°C and 34 percent relative humidity. The values obtained are listed in the table below.

Development occurred at 20°C for 5 min. in a developing solution having the following composition:

|                                  |           |
|----------------------------------|-----------|
| water                            | 800 ccs   |
| p-monomethylaminophenol sulphate | 1.5 g     |
| sodium sulphite (anhydrous)      | 50 g      |
| hydroquinone                     | 6 g       |
| sodium carbonate (anhydrous)     | 32 g      |
| potassium bromide                | 2 g       |
| water to make                    | 1000 ccs. |

Table

| Compound added | Fresh material |           |       |     | Incubated material |           |       |     |
|----------------|----------------|-----------|-------|-----|--------------------|-----------|-------|-----|
|                | Speed          |           | Speed |     | Speed              |           | Speed |     |
|                | Fog            | Gradation | I     | II  | Fog                | Gradation | I     | II  |
| none           | 0.09           | 1.97      | 100   | 100 | 0.71               | 1.62      | 95    | 85  |
| compound 22    | 0.09           | 1.95      | 100   | 93  | 0.29               | 1.81      | 129   | 110 |
| compound 23    | 0.06           | 2.04      | 89    | 89  | 0.19               | 1.80      | 151   | 112 |

The following examples illustrate the stabilizing and fog-inhibiting action of the compounds corresponding to the above general formula. In these examples, the values I and II given for the speed are relative values corresponding with density 0.1 above fog and density 1 above fog respectively; the values of 100 are given to

30 35

## EXAMPLE 2

Example 1 was repeated with the difference that the emulsion was divided into four aliquot portions to which the compounds listed in the table below were added in the concentration given. The sensitometric results obtained are listed in the following table.

| Compound added per kg of emulsion                  | fog  | Fresh material |       |     |      | Incubated material |                |     |    |
|----------------------------------------------------|------|----------------|-------|-----|------|--------------------|----------------|-----|----|
|                                                    |      | grad-<br>ation | speed | I   | II   | fog                | grad-<br>ation | I   | II |
| none                                               | 0.07 | 1.30           | 100   | 100 | 0.43 | 1.17               | 191            | 126 |    |
| 1 millimole of compound 11                         | 0.09 | 1.47           | 112   | 120 | 0.19 | 1.34               | 138            | 126 |    |
| 2 millimoles of compound 12                        | 0.08 | 1.36           | 102   | 110 | 0.23 | 1.25               | 148            | 129 |    |
| 1 millimole of 1-ethyl-2-(2-pyridyl)-benzimidazole | 0.08 | 1.41           | 66    | 52  | 0.18 | 1.30               | 62             | 81  |    |

the emulsions comprising no stabilizer of the invention.

## EXAMPLE 1

A conventional photographic gelatino silver bromo-iodide emulsion (4.5 mole % iodide) comprising per kg an amount of silver halide equivalent to 50 g of silver nitrate was divided into three portions. To two of these emulsion portions was added a compound as listed in

55

As can be seen from these results, compounds similar to those of the invention but containing no water-solubilizing group reduce the fogging tendency but at the cost of a considerable reduction of the sensitivity.

## EXAMPLE 3

Example 1 was repeated with the difference that the emulsion was divided into four aliquot portions to which the compounds listed in the table below were added in the concentration given.

The following sensitometric results were attained.

| Compound added per kg of emulsion | fog  | Fresh material |       |     |      | Incubated material |                |     |    |
|-----------------------------------|------|----------------|-------|-----|------|--------------------|----------------|-----|----|
|                                   |      | grad-<br>ation | speed | I   | II   | fog                | grad-<br>ation | I   | II |
| none                              | 0.08 | 1.67           | 100   | 100 | 0.43 | 1.33               | 141            | 123 |    |
| 4 millimoles of compound 1        | 0.08 | 1.52           | 93    | 89  | 0.21 | 1.35               | 148            | 126 |    |
| 2 millimoles of compound 2        | 0.07 | 1.59           | 102   | 98  | 0.21 | 1.52               | 132            | 120 |    |
| 2 millimoles of compound 3        | 0.09 | 1.73           | 59    | 60  | 0.27 | 1.62               | 105            | 89  |    |

## EXAMPLE 4

Example 1 was repeated with the difference that the emulsion was divided into seven aliquot portions to which the compounds listed in the table below were added in a concentration of 1 millimole per kg of emulsion.

The following sensitometric results were attained.

| Compound added per kg of emulsion  | fog  | Fresh material |       |     | fog  | Incubated material |       |     |
|------------------------------------|------|----------------|-------|-----|------|--------------------|-------|-----|
|                                    |      | gradation      | speed | I   |      | gradation          | speed | I   |
| none                               | 0.36 | 1.74           | 100   | 100 | 1.08 | 1.40               | 78    | 65  |
| compound 7                         | 0.12 | 2.14           | 89    | 105 | 0.31 | 1.71               | 107   | 100 |
| compound 8                         | 0.16 | 1.40           | 81    | 69  | 0.42 | 1.36               | 85    | 69  |
| compound 4                         | 0.13 | 1.75           | 67    | 74  | 0.38 | 1.66               | 85    | 83  |
| compound 5                         | 0.12 | 2.22           | 67    | 76  | 0.17 | 2.16               | 71    | 79  |
| compound 10                        | 0.10 | 2.12           | 42    | 51  | 0.10 | 1.96               | 50    | 57  |
| 2,6-bis(2-benzimidazolyl)-pyridine | 0.08 | 1.90           | 27    | 28  | 0.10 | 1.82               | 30    | 29  |

From the results it appears that compounds similar to those of the invention but containing no water-soluble group also reduce the fogging tendency of the emulsion but at a cost of a considerable reduction of the sensitivity.

## EXAMPLE 5

Example 1 was repeated with the difference that the emulsion was divided into two aliquot portions. To one of these portions was added 1 millimole of compound 24 whereas to the other emulsion portion no compound according to the invention was added.

The following sensitometric results were attained.

| Compound added | fog  | Fresh material |       |     | fog  | Incubated material |       |     |
|----------------|------|----------------|-------|-----|------|--------------------|-------|-----|
|                |      | gradation      | speed | I   |      | gradation          | speed | I   |
| none           | 0.09 | 1.67           | 100   | 100 | 0.65 | 1.14               | 144   | 93  |
| compound 24    | 0.08 | 1.62           | 81    | 87  | 0.29 | 1.36               | 138   | 117 |

## EXAMPLE 6

Example 5 was repeated but now compound 9 was used instead of compound 24.

The following sensitometric results were attained.

| Compound added | fog  | Fresh material |       |     | fog  | Incubated material |       |    |
|----------------|------|----------------|-------|-----|------|--------------------|-------|----|
|                |      | gradation      | speed | I   |      | gradation          | speed | I  |
| none           | 0.13 | 1.90           | 100   | 100 | 1.31 | 1.50               | 65    | 61 |
| compound 9     | 0.09 | 2.03           | 91    | 85  | 0.38 | 1.75               | 69    | 85 |

## EXAMPLE 7

A washed negative gelatin silver bromoiodide emulsion (average grain size of the silver halide : 0.8  $\mu$ ) the silver halide of which consists of 94.5 mole percent of silver bromide and 5.5 mole percent of silver iodide, was ripened at 45°C. The emulsion ready for coating contained per kg 50 g of silver halide, 75 g of gelatin, 30 mg of optical sensitizer corresponding to the following structural formula:



50 mg of 5-methyl-7-hydroxy-s-triazolo[1,5-a]pyrimidine as a stabilizer, and 500 mg of saponine as a wetting agent.

This emulsion was divided into two aliquot portions A and B and to one of them (B) was added 500 mg of compound 8 per kg of emulsion.

The emulsion portions were both applied to cellulose triacetate supports and dried.

The materials A and B obtained were both exposed in the same circumstances through a grey wedge and

5

20

25

30

40

55

60

65

developed for 8 min. at 20°C in a developer having the following composition:

|                                 |         |
|---------------------------------|---------|
| water                           | 750 ccs |
| N-methyl-p-aminophenyl sulphate | 2g      |
| anhydrous sodium sulphite       | 100g    |
| hydroquinone                    | 5g      |
| granular borax                  | 2g      |
| water to make                   | 100 ccs |

The fog produced in the freshly prepared materials and identical materials that have been stored for 10 days at 57°C and 34 percent relative humidity is listed in the following table. The gradation and speed of the fresh materials and incubated materials have remained the same.

| Material   | Fog produced in |                     |
|------------|-----------------|---------------------|
|            | Fresh materials | Incubated materials |
| Material A | 0.06            | 0.24                |
| Material B | 0.05            | 0.13                |

## EXAMPLE 8

A silver bromoiodide emulsion as described in example 7 was prepared and divided into two aliquot portions A and B. To one of these (B) were added 30 mg of compound 10 per kg of emulsion.

The emulsions were both applied to cellulose triacetate supports and dried.

The materials A and B obtained were both exposed in the same circumstances through a grey wedge and then rapidly developed (for 1 min. only) at an elevated temperature (36°C) in a developer having a pH of 10.4 and comprising per litre 36 g of sodium sulphite, 10.5 g of hydroquinone, 0.25 g of 1-phenyl-3-pyrazolidinone, 4 g of sodium bromide, 20 g of potassium carbonate and 2.2 g of sodium hydroxide.

The fog produced in the material comprising as stabilizer only 5-methyl-7-hydroxy-s-triazolo[1,5-a]pyrimidine namely 0.18 was markedly higher than

that produced in the material comprising a compound according to the invention in addition to the said triazolopyrimidine namely 0.11.

The gradation and the speed remained practically unchanged.

#### EXAMPLE 9

A conventional photographic gelatino silver bromo-iodide emulsion (4.5 mole percent iodide) comprising per kg an amount of silver halide equivalent to 50 g of silver nitrate was divided into 4 portions. To 3 of these portions was added a compound as listed in the table below in the concentration given. The emulsions were coated on a conventional support and dried.

The values of speed, gradation and fog of the materials formed were determined shortly after preparation and after incubation for 5 days at 57°C and 34 percent relative humidity. The values obtained are listed in the table below.

Exposure occurred through a step-wedge with constant 0.15.

Development occurred at 20°C for 5 min. in a developer solution having a composition as given in Example 1.

| Compound added per kg of emulsion | fog  | Fresh material |     |       |      | Incubated material |     |       |  |
|-----------------------------------|------|----------------|-----|-------|------|--------------------|-----|-------|--|
|                                   |      | gradation      |     | speed |      | gradation          |     | speed |  |
|                                   |      | I              | II  |       |      | I                  | II  |       |  |
| none                              | 0.13 | 1.73           | 100 | 100   | 0.66 | 1.28               | 204 | 83    |  |
| 150 mg of (1)                     | 0.13 | 1.73           | 107 | 78    | 0.25 | 1.42               | 195 | 135   |  |
| 1 millimole of compound 29        | 0.12 | 1.85           | 129 | 102   | 0.43 | 1.63               | 200 | 135   |  |
| 2 millimoles of compound 29       | 0.11 | 1.83           | 115 | 93    | 0.22 | 1.62               | 200 | 141   |  |

#### (1) 5-methyl-7-hydroxy-s-triazolo-[1,5-a]pyrimidine.

We claim:

1. Photographic material comprising a support and at least one light-sensitive silver halide emulsion layer comprising in said emulsion layer and/or in at least one water-permeable layer coated at the same side of the support as the said emulsion layer at least one heterocyclic bidentate reagent for silver corresponding to the following general formula:



wherein

R stands for hydrogen or a one to four carbon atom alkyl group,

Z represents the atoms necessary to complete an imidazole nucleus, a benzimidazole nucleus, a naph-

thimidazole nucleus, an imidazopyridine nucleus, an imidazole nucleus, a pyrazole nucleus, a triazole nucleus or a tetrazole nucleus,

A stands for a single chemical bond, an alkylene group containing from one to four carbon atoms in a carbon to carbon chain, including alkylene interrupted by oxygen or a -N(R) group, wherein R stands for hydrogen or a one to four carbon atom alkyl group, arylene, alkenylene and -S-alkylene-S- or -S-alkylene, the alkylene groups of which will contain from one to four carbon atoms in a carbon to carbon chain and can be interrupted by oxygen or an -N(R)- group wherein R stands for hydrogen and a one to four carbon atom alkyl group.

X stands for a 5- or 6-membered heterocycle, said heterocycle comprising the grouping =N—, and wherein a carboxyl group or sulpho group in acid or salt form is linked directly or indirectly to the grouping Z and/or X and/or A, said bidentate reagent being present in a fog-inhibiting amount.

2. Photographic material according to claim 1, wherein X stands for an imidazole nucleus, a benzimidazole nucleus, a naphthimidazole nucleus, an

imidazopyridine nucleus, an imidazoline nucleus, a pyrazole nucleus, a pyridine nucleus, a quinoline nucleus, a thiazole nucleus, a triazole nucleus or a tetrazole nucleus.

3. Photographic light-sensitive silver halide material according to claim 1, wherein said heterocyclic bidentate reagent for silver is present in the light-sensitive silver halide emulsion layer in an amount between 0.2 and 30 millimoles per mole of silver halide.

4. Photographic light-sensitive silver halide material according to claim 1, wherein said material also comprises a hydroxytriazolopyrimidine stabilizer.

5. Photographic light-sensitive silver halide material according to claim 1, wherein said material also comprises a polyoxyalkylene development accelerator.

6. Photographic light-sensitive silver halide material according to claim 1, wherein said emulsion layer is a gelatino silver halide emulsion layer.

\* \* \* \* \*